

## 1

3,582,323

### ALUMINUM-IRON ALLOY FOR EXHAUST VALVES OF INTERNAL COMBUSTION ENGINES

John C. Sawyer and Charles F. Barth, Cleveland, Ohio,  
assignors to TRW Inc., Cleveland, Ohio

No Drawing. Filed Nov. 17, 1967, Ser. No. 683,816

Int. Cl. C22c 37/10

U.S. Cl. 75—124

1 Claim

#### ABSTRACT OF THE DISCLOSURE

Iron-aluminum alloys particularly useful in exhaust valves for internal combustion engines, the alloys having an iron-aluminum matrix containing from 30 to 50 atomic percent aluminum, and one or more hardening elements totaling not in excess of 6 atomic percent.

#### BACKGROUND OF THE INVENTION

##### Field of the invention

This invention is directed to an improved alloy system having excellent strength properties at elevated temperatures and improved lead oxide corrosion resistance, the alloy having a matrix consisting both of iron and aluminum having sufficient aluminum present to favor the production of the intermetallic compound FeAl, and containing one or more hardening elements in amounts totaling not in excess of about 6 atomic percent, the hardening elements being such materials as zirconium, molybdenum, carbon, titanium, vanadium, tantalum and lanthanum.

##### Description of the prior art

There are numerous criteria involved in the choice of suitable materials for exhaust valves. These have been well stated in the chapter entitled "The Selection of Material for Engine Valves" prepared by the American Society for Metals Committee on Engine Valves, appearing at pages 626 to 634, inclusive, of "Metals Handbook," Eighth edition, volume 1. As detailed in that article, typical wrought and cast alloys used for valves may include ferritic steels, sigma phase alloys, austenitic alloys or nickel alloys. For the most part, however, these alloys contain no aluminum or those that do contain very small amounts.

#### SUMMARY OF THE INVENTION

The present invention provides an iron-aluminum matrix useful for exhaust valves in internal combustion engines because of its low density, excellent corrosion resistance, hot hardness, mechanical strength, and low cost. The matrix consists of an iron-aluminum binary alloy containing from 30 to 50 atomic percent aluminum (17.1 to 32.6 weight percent), the amount of aluminum present being conducive to the formation of the intermetallic compound FeAl. Studies have indicated that the oxides formed at elevated temperatures on alloys of this type have a relatively high resistance to lead oxide attack. However, alloys having high aluminum contents are frequently brittle and lack the hot hardness and mechanical strength required for use in valves operating at temperatures of 1200° to 1600° F. These problems have now been satisfactorily met by control of processing variables and by the addition of suitable hardening elements in controlled amounts, the hardening elements being one or more of the

## 2

following group: zirconium, molybdenum, carbon, titanium, vanadium, tantalum and lanthanum. We have found that when these hardening elements are added in amounts totaling not in excess of about 6 atomic percent, the hot hardness and mechanical strength properties of the iron-aluminum matrix are improved to the extent that they are completely useful in exhaust valves operating at elevated temperatures.

#### DESCRIPTION OF THE PREFERRED EMBODIMENTS

The alloy of the present invention, in its broader aspects, contains from 50 to 70 atomic percent iron, from 30 to 50 atomic percent aluminum, and one or more hardening elements, these hardening elements including up to 1 atomic percent zirconium, up to 1.5 atomic percent carbon, up to 5 atomic percent lanthanum, up to 5 atomic percent vanadium, up to 5 atomic percent tantalum, up to 5 atomic percent molybdenum and up to 5 atomic percent titanium. In the preferred form of the invention, the matrix contains from 38 to 42 atomic percent aluminum, the balance being iron, and the hardening elements include the addition of from 0.1 to 1.0 atomic percent zirconium, from 0.05 to 1.0 atomic percent carbon, from 1 to 4 atomic percent vanadium, from 1 to 4 atomic percent tantalum, from 1 to 4 atomic percent molybdenum, from 0.1 to 4 atomic percent titanium and from 0.1 to 4 atomic percent lanthanum.

The alloys of the present invention have yield strengths of at least 30,000 p.s.i. at 1400° F., and a lead oxide corrosion loss not in excess of 25 grams per square decimeter per hour at 1675° F. The lead oxide corrosion test is a laboratory bench-type test employed for evaluation of corrosion resistance of exhaust valve alloys, and involves preparing a specimen of the test alloy, 0.444 inch in diameter by 0.444 inch in length and placing this specimen in a magnesia crucible with 40 grams of lead oxide, and heating to 1675° F. for one hour. The specimen is then cooled to room temperature, cleaned and weighed. The loss in weight expressed per unit area represents a measure of the relative corrosion resistance of the alloy.

The strengthening of the iron-aluminum matrix can be attained through alloy additions of either molybdenum, tantalum or vanadium or through further additions based on titanium, carbon and zirconium in combination with the preceding additives. These additives appear to provide improved age hardening properties to the alloys. The following table illustrates the results obtained when varying amounts of additives were added to an iron-aluminum matrix containing 40 atomic percent aluminum:

TABLE I

| Alloy addition | Atomic percent | Weight percent | Brinell Hardness                              |                                           |  |
|----------------|----------------|----------------|-----------------------------------------------|-------------------------------------------|--|
|                |                |                | 3,000 kg. load,<br>10 mm. ball,<br>room temp. | 750 kg. load,<br>5 mm. ball,<br>1,400° F. |  |
| V-----         | 2.0            | 2.3            | 362                                           | 110                                       |  |
| V-----         | 4.0            | 4.6            | 372                                           | 149                                       |  |
| Ta-----        | 2.0            | 7.7            | 362                                           | 131                                       |  |
| Ta-----        | 4.0            | 14.7           | 382                                           | 216                                       |  |
| Mo-----        | 2.0            | 4.3            | 362                                           | 112                                       |  |
| Mo-----        | 4.0            | 8.4            | 352                                           | 163                                       |  |
| Mo, C          | 2.0, 0.5       | 4.3, 0.13      | 372                                           | 160                                       |  |
| Ti, Zr, C      | 1.0, 0.2, 0.3  | 1.3, 0.5, 0.08 | 290                                           | 125                                       |  |

The mechanical properties of some of the alloy compositions, showing the improvements achieved by the vari-

ous alloying additions are summarized in the following table:

The best overall properties achieved in alloys produced according to the present invention occur in those alloys

TABLE II

| Heat No. | Nominal composition, atomic percent | Condition                                                           | Mechanical properties at 1,400° F., 0.2% offset |                          |                    |
|----------|-------------------------------------|---------------------------------------------------------------------|-------------------------------------------------|--------------------------|--------------------|
|          |                                     |                                                                     | Yield strength, K s.i.                          | Tensile strength, K s.i. | Percent elongation |
| 3        | Fe-38Al                             | { As extruded<br>Aged 100 hr. at 1,600° F.                          | 21<br>19                                        | 23<br>23                 | 80<br>122          |
| 9        | Fe-46Al-1Ti-0.2Zr-0.2C              | As extruded                                                         | 22                                              | 30                       | 57                 |
| 9A       | Fe-38Al-2Ti-0.1Zr-0.6C              | { As extruded<br>Solution treated 2 hrs. at 2,000° F., oil quenched | 24<br>34                                        | 32<br>39                 | 52<br>50           |
| 10       | Fe-41Al-2-Mo2Ti-0.2Zr-0.9C          | { As extruded<br>Solution treated 2 hrs. at 2,000° F., oil quenched | 34<br>35, 247                                   | 45<br>—, 247.2           | 71<br>140, 280     |
| 11       | Fe-41Al-2Mo-2Ti-0.1Zr-1C            | { As extruded<br>Solution treated 2 hrs. at 2,000° F., oil quenched | 27<br>31                                        | 35<br>39                 | 74<br>80           |

<sup>1</sup> Premature fracture.

<sup>2</sup> Specimen tested at the normally used crosshead speed of 0.1 inch per minute, the other data were obtained at a slower cross-head speed of 0.01 inch per minute.

The hot hardness of the alloys was evaluated using samples  $\frac{1}{2}$  inch in diameter by  $\frac{1}{2}$  inch long. The samples were prepared for hot hardness evaluation in the as extruded condition and after a stabilization treatment at 1800° F. for 16 hours. As evident from the following table, the stabilization treatment increases the hot hardness of the extruded alloy by approximately 20% in most instances.

which contain the combination of molybdenum, titanium, carbon, and zirconium. These alloys have yield strengths of about 47,000 p.s.i. at 1400° F., and a lead oxide corrosion resistance of 11 to 12 grams per square decimeter per hour at 1675° F.

The relatively low cost of the alloys of the present invention makes it possible to produce the entire valve structure from the alloys and still remain competitive with valve alloys containing substantial amounts of chromium. If desired, however, the application of the alloy can be restricted to facing of the valve seat or other portions of the valve which are subjected to high temperatures and severe lead oxide corrosion problems.

It should be evident that various modifications can be made to the described embodiments without departing from the scope of the present invention.

We claim as our invention:

1. An exhaust valve for an internal combustion engine composed at least in part of an iron-aluminum matrix consisting essentially of from 38 to 42 atomic percent aluminum, balance iron, and at least one hardening element selected from the group consisting of 0.1 to 1.0 atomic percent zirconium, 0.05 to 1.0 atomic percent carbon, 1 to 4 atomic percent vanadium, 1 to 4 atomic percent tantalum, 1 to 4 atomic percent molybdenum, 0.1 to 4 atomic percent titanium, and 0.1 to 4 atomic percent lanthanum.

45

#### References Cited

#### UNITED STATES PATENTS

|    |           |         |           |        |
|----|-----------|---------|-----------|--------|
| 50 | 2,579,369 | 12/1951 | Dawe      | 75—124 |
|    | 2,604,455 | 7/1952  | Reynolds  | 75—124 |
|    | 2,946,676 | 7/1960  | Brennan   | 75—124 |
|    | 3,303,561 | 2/1967  | Cabane    | 75—124 |
|    | 3,386,819 | 1/1968  | Cabane    | 75—124 |
|    | 3,420,660 | 1/1969  | Kawahatta | 75—124 |

55 HYLAND BIZOT, Primary Examiner

U.S. Cl. X.R.

75—123

| Heat No. | Nominal composition, atomic percent | Brinell Hardness                    |                        |
|----------|-------------------------------------|-------------------------------------|------------------------|
|          |                                     | 750 kg. load, 1,400° F. as extruded | 5 mm. ball, stabilized |
| 1        | Fe-40Al-1Mo                         | 82                                  |                        |
| 3        | Fe-38Al                             | 78                                  | 98                     |
| 4        | Fe-41Al-2Mo-0.3C                    | 80                                  | 10 <sup>2</sup>        |
| 5        | Fe-42Al-2Ta                         | 82                                  | 104                    |
| 6        | Fe-40Al-4Mo-0.2C                    | 75                                  | 103                    |
| 7        | Fe-40Al-2Mo-0.6C                    | 93                                  | 101                    |

Several samples each of the various alloys were subjected to 1675° F. lead oxide corrosion test in the as extruded condition. The average values attained in the lead oxide corrosion test are given in the following table:

TABLE IV

| Heat No. | Nominal composition, atomic percent | Average PbO loss, gm./dm. <sup>2</sup> /hr. at 1,675° F. | PbO loss, gm./dm. <sup>2</sup> /hr. at 1,675° F. |      |
|----------|-------------------------------------|----------------------------------------------------------|--------------------------------------------------|------|
|          |                                     |                                                          | 14.9                                             | 14.0 |
| 1        | Fe-40Al-1Mo                         | 14.9                                                     |                                                  |      |
| 3        | Fe-38Al                             | 14.0                                                     |                                                  |      |
| 4        | Fe-41Al-2Mo-0.3C                    | 18.5                                                     |                                                  |      |
| 5        | Fe-42Al-2Ta                         | 23.0                                                     |                                                  |      |
| 6        | Fe-40Al-4Mo-0.2C                    | 13.2                                                     |                                                  |      |
| 7        | Fe-40Al-2Mo-0.6C                    | 14.0                                                     |                                                  |      |
| 9        | Fe-46Al-1Ti-0.2Zr-0.2C              | 10.8                                                     |                                                  |      |
| 9A       | Fe-38Al-2Ti-0.1Zr-0.6C              | 12.4                                                     |                                                  |      |
| 10       | Fe-41Al-2Mo-2Ti-0.2Zr-0.9C          | 11.8                                                     |                                                  |      |
| 11       | Fe-41Al-2Mo-2Ti-0.1Zr-1C            | 12.1                                                     |                                                  |      |